

April 1, 1969

K. HASS ET AL

3,436,324

CORROSION-ENDANGERED PARTS OF APPARATUS USED IN ALKALI  
METAL CHLORIDE ELECTROLYSIS HAVING PROTECTIVE  
COVERING OF POST-CHLORINATED PVC

Filed May 2, 1966

FIG. 1.



FIG. 2.



INVENTORS

KARL HASS  
WALTER KOLHAGEN  
GÜNTHER CZEHOVSKY  
HANS-EWALD KONERMANN

BY

*Surgess, Dinklage + Sprung*

ATTORNEYS.

## 1

3,436,324

## CORROSION-ENDANGERED PARTS OF APPARATUS USED IN ALKALI METAL CHLORIDE ELECTROLYSIS HAVING PROTECTIVE COVERING OF POST-CHLORINATED PVC

Karl Hass, Niederkassel, Walter Kolhagen, Cologne-Dellbrück, Gunther Czechovsky, Niederkassel, and Hans-Ewald Konermann, Oberlar, Germany, assignors to Dynamit Nobel Aktiengesellschaft, Troisdorf, Bezirk Cologne, Germany

Filed May 2, 1966, Ser. No. 548,028

Claims priority, application Germany, Apr. 30, 1965,  
D 47,153

Int. Cl. B01k 1/00

U.S. Cl. 204—128

8 Claims

The subject of the invention is the use of special types of post-chlorinated polyvinyl chloride as a coating material for corrosion-endangered parts of apparatus used in alkali metal chloride electrolysis.

It is in the prior art to manufacture out of metallic materials, conduits having a protective lining for parts of apparatus used in alkali metal chloride electrolysis, and to protect the surface with material that resists the action of the aggressive liquids and gases in the electrolysis cell, such as rubber or plastics for example. It is also in the prior art to use tubing and sleeves that are made wholly from ceramic or like material, such as porcelain and glass. Also known is the manufacture of the above-mentioned apparatus parts partially from solid plastics, and also in one layer or in a plurality of layers from plastics of various kinds with and without mechanical reinforcement by inorganic and organic fibrous materials. Disadvantages of the materials listed consist mainly in the fact that the coatings become separated from the structure covered, and also they often do not adequately resist the chemical attack.

Ceramic material generally offers quite good chemical resistance under the conditions of alkali metal chloride

TABLE I

| Experiment No. | Material                                    | Time (days) | Temp., °C. | Change in O.D. | State after Removal                                                                  |
|----------------|---------------------------------------------|-------------|------------|----------------|--------------------------------------------------------------------------------------|
| 1a             | Polyethylene (unfilled)                     | 60          | 83         | +1.5%          | Surface smooth, many individual bubbles protruding as much as 3 mm.                  |
| 1b             | Polyethylene (stabilized with carbon black) | 143         | 85         | +2.4%          | Surface irregular, with bumps up to 4 mm. beyond diameter.                           |
| 1c             | do                                          | 155         | 83         | +9.4%          | Surface textured; layer 0.6 mm. thick spalled off.                                   |
| 1d             | Polypropylene                               | 155         | 83         | -2.6%          | Loss of substance due to spalling off of thin layers 0.1 mm. thick.                  |
| 1e             | do                                          | 143         | 85         | -1.7%          | Do.                                                                                  |
| 1f             | Polyvinyl chloride                          | 126         | 84         | +7.5%          | Uniform thickening over entire surface subject to attack. Surface rough and brittle. |
| 1g             | do                                          | 160         | 85         | +8.6%          | Do.                                                                                  |
| 1h             | Polyvinyl chloride (post-chlorinated)       | 155         | 83         | +0.2%          | Surface uniformly smooth, unaltered.                                                 |
| 1i             | do                                          | 143         | 85         | +0.2%          | Do.                                                                                  |

electrolysis, but its relatively low resistance to breakage and thermal shock is disadvantageous. Furthermore, the plastics hitherto used either in solid form or as coatings are subject, after relatively long operation under the said conditions, to alterations affecting the surfaces (so that, for example, a tube carried movably in a sealing gland can no longer be moved) and to alterations which gradually lead to the destruction of the entire material.

It has now been found that, with the avoidance of the above-described disadvantages, especially post-chlorinated PVC with a chlorine content of at least about 64 wt.

## 2

percent, for example 64–70 wt. percent, and in which about 50 to 90 wt. percent and preferably about 60 to 80 wt. percent of the additional chlorine introduced by post-chlorination is in 1,2-dichloroethylene units, can be used advantageously as coating material for corrosion-endangered parts of apparatus used in alkali metal chloride electrolysis.

The advantages of the use, according to the invention, of the described post-chlorinated types of PVC, lie both in the good thermal stability and in the good resistance to breakage of such coatings, combined with outstanding corrosion resistance. The said coatings are furthermore susceptible of welding and cementing. They can also be cut and machined, even after application.

With the material described, corrosion-endangered tubing, covers for the power lines to the graphite anodes, lid coatings, bath and vat linings and other parts of alkali metal chloride electrolysis equipment can be coated, as well as other products.

The coating material of the invention may contain the conventional substances to improve workability. The semi-products which are used for the manufacture of the coatings can be made by plastics manufacturing methods of the prior art.

The use according to the invention of the chlorine-containing thermoplastics described is illustrated by the following examples:

## Example 1

Used as protective tubing for the conductors connected to the graphite anodes of equipment used in sodium chloride electrolysis.

The conductors of the graphite anodes were covered with pieces of plastic tubing with a 4 mm. wall thickness and a 40 mm. outside diameter, and were exposed to the effects of a sodium chloride electrolysis at the stated temperatures and times.

1a to 1g: Examples for comparative purposes.

1h to 1i: Examples of the use of various types of post-chlorinated PVC.

The post-chlorinated polyvinyl chloride used in Example 1 was produced as follows: A suspension PVC with a K value of 68 was brought up by post-chlorination to a chlorine content of 67.2%. 69% of the chlorine is disposed in 1,2-dichloroethylene units (the 1,2-dichloroethylene unit content was determined by measurement of the nuclear resonance spectrum). After the addition of 3 wt. percent of Ba-Cd laurate, 2 wt. percent of a lubricant commercially obtainable under the name of "E-Wax" and 0.5 wt. percent of calcium stearate, the material was extruded at 190° C. into tubes of the specified size.

**3**  
Example 2

Used as bath lining:  
2a to 2b: Tests for comparison  
2c: Use of a type of post-chlorinated PVC.

TABLE 2

| Experiment No. | Material                                              | Time<br>(days) | Temp.,<br>° C. | Change in<br>O.D. | Findings                                                 |
|----------------|-------------------------------------------------------|----------------|----------------|-------------------|----------------------------------------------------------|
| 2a             | Fibercast (epoxy resin) sheet                         | 40             | 83             | -6.4%             | Loss of material, crumbly surface.                       |
| 2b             | Polyethylene sheet (stabilized with<br>carbon black). | 35             | 78             | +4.2%             | Surface textured, occasional closed<br>bubbles bleached. |
| 2c             | Polyvinyl chloride sheet (post-chlori-<br>nated).     | 30             | 75             | +0.04%            | Edges unaltered and smooth surface.                      |

The post-chlorinated PVC used in Example 2 was produced as follows: A suspension PVC with a K value (H. 15 Fikentscher Cellulosechemie, 13, 1932, p. 58) of 60 was brought up by post-chlorination to a chlorine content of 65.8%. 75.5% of the chlorine was attached in units of 1,2-dichloroethylene (the 1,2-dichloroethylene unit content was determined by measuring the nuclear resonance 20 spectrum). The material after the addition of 3 wt. percent of Ba-Cd laurate, 1 wt. percent of titanium dioxide and 0.5 wt. percent of Ca stearate, was rolled to a sheet 0.5 mm. thick and then pressed into sheets 4 mm. thick at 190° C.

Thus, the invention provides an electrolysis cell for electrolysis of alkali metal chloride comprising equipment including a tank for holding an alkali metal chloride bath for electrolyzing, electrodes disposed in the tank, conduit for conveyance of electrolysis material, and conductors connected to said electrodes, and an alkali metal chloride bath for electrolysis in the tank. According to the invention, a least part of the equipment is provided with a protective covering consisting essentially of post-chlorinated polyvinyl chloride polymer.

The invention is further described in reference to the accompanying drawing, wherein:

FIG. 1 is a schematic representation of an electrolysis diaphragm cell according to the invention.

A tank 1 is provided with a protective covering 2, and is outfitted with lid 10, which is provided with a protective covering 12. A sodium chloride brine bath 20 is contained within the tank, and anode 4 and cathode 5 are immersed in the tank. The cathode is covered by a diaphragm 6. The anode and the cathode are serviced by conductors insulated by a protective covering according to the invention. The conductor 14 which is connected to the anode 4 is provided with protective covering 13; the conductor 15 which is connected to the cathode 5 is protected by protective covering 7. Bushings 3 and 9 are provided where the conductors pass through the tank wall and the wall of the lid. These bushings can be formed of post-chlorinated polyvinyl chloride according to the invention. Conduit 16 is provided for withdrawal of chlorine from the cell, and is provided with a protective lining 17; similarly, conduit 8 is provided for withdrawing hydrogen from the cathode, and is also provided with a protective lining (not shown). The various protective coverings and linings mentioned are of post-chlorinated polyvinyl chloride according to the invention.

FIG. 2 is a schematic representation of an electrolysis mercury cell according to the invention.

The description, apart from constructural differences, corresponds with that given for FIG. 1, except that 4 being the graphite anode and 5 the mercury cathode. 21 is for the introduction of the brine.

The post-chlorinated polyvinyl chloride used in the invention has a chlorine content of between about 64 and 70 wt. percent and in which about 50 to 90 wt. percent of the additional chlorine introduced by post-chlorination is in 1,2-dichloro-ethylene units. It can be produced by the procedure disclosed in the Belgian Patent 654,377, corresponding with our pending U.S.-application Ser. No. 403,949, filed Oct. 14, 1964, now Patent No. 3,362,896. The 1,2 - dichloro-ethylene units can be determined by

measurement of the nuclear resonance spectrum. This method is described in Ang. Chemie 77 (1965) pp. 1124-34 by H. J. Harewood. The post-chlorinated polyvinyl chloride can be rolled at 170-190° C. The thermal sta-

bility of the described material is superior to other known types.

The invention finds application for all processes wherein alkali chlorides are electrolyzed, and chlorine is produced.

While the invention has been described with respect to particular embodiments thereof, these embodiments are merely representative and do not serve to determine the limits of the invention.

What is claimed is:

1. Electrolysis cell for electrolysis of alkali metal chloride comprising equipment adapted to contact said alkali metal chloride and reaction products produced therefrom comprising a corrosive reaction environment including a tank for holding an alkali metal chloride bath for electrolyzing, electrodes disposed in the tank, conduit for conveyance of electrolysis material, and conductors connected to said electrodes, at least part of said equipment being susceptible to corrosion and having a protective covering consisting essentially of post-chlorinated polyvinyl chloride polymer.

2. Electrolysis cell according to claim 1, said post-chlorinated polyvinyl chloride having a chlorine content of about 64-70 wt. percent, and about 50-90 wt. percent of the additional chlorine introduced by post-chlorination being in 1,2-dichloroethylene units.

3. Electrolysis cell according to claim 2, wherein the cell is lined with said protective covering.

4. Electrolysis cell according to claim 3, wherein said conductors are protected with said protective covering.

5. Electrolysis cell according to claim 4, wherein said conduit is lined with said protective covering.

6. Electrolysis cell according to claim 2, wherein said conductors are protected with said protective covering.

7. Electrolysis cell according to claim 2, wherein said conduit is lined with said protective covering.

8. A process for production of chlorine comprising electrolyzing alkali metal chloride in an electrolysis cell thereby producing a corrosive reaction environment, said cell including equipment exposed to the corrosive reaction environment, said equipment including a tank holding the alkali metal chloride bath, electrodes disposed in the tank, conduit for conveyance of electrolysis material, and conductors connected to said electrodes, at least part of said equipment being susceptible to corrosion and having a protective covering consisting essentially of post-chlorinated polyvinyl chloride polymer.

**References Cited**

**UNITED STATES PATENTS**

2,764,542 9/1956 Pullen \_\_\_\_\_ 204-268 XR  
2,989,450 6/1961 Maylott et al. \_\_\_\_\_ 204-94

**OTHER REFERENCES**

Evans, Tank Linings, Metal Industry, July 29, 1949, pp. 86-88.

Evans, J.E.T.S., vol. 24, pp. 129-143, 1948-49.

70 JOHN H. MACK, Primary Examiner.

D. R. JORDAN, Assistant Examiner.

U.S. Cl. X.R.

75 204-242, 219, 278; 220-63